



US010791756B2

(12) **United States Patent**  
**Zuchuat et al.**

(10) **Patent No.:** **US 10,791,756 B2**  
(b4) **Date of Patent:** **Oct. 6, 2020**

(54) **RECONSTITUTED TOBACCO SHEETS AND RELATED METHODS**

(71) Applicant: **PHILIP MORRIS PRODUCTS S.A.**,  
Neuchatel (CH)

(72) Inventors: **Fabien Zuchuat**, Sion (CH); **Alen Kadircic**, Orpund (CH)

(73) Assignee: **Philip Morris Products S.A.**,  
Neuchatel (CH)

(\*) Notice: Subject to any disclaimer, the term of this patent is extended or adjusted under 35 U.S.C. 154(b) by 726 days.

(21) Appl. No.: **15/305,131**

(22) PCT Filed: **Jun. 22, 2015**

(86) PCT No.: **PCT/EP2015/063979**

§ 371 (c)(1),  
(2) Date: **Oct. 19, 2016**

(87) PCT Pub. No.: **WO2015/197554**

PCT Pub. Date: **Dec. 30, 2015**

(65) **Prior Publication Data**

US 2017/0035095 A1 Feb. 9, 2017

(30) **Foreign Application Priority Data**

Jun. 24, 2014 (EP) ..... 14173740

(51) **Int. Cl.**

*A24B 3/14* (2006.01)  
*A24B 15/12* (2006.01)  
*A24B 3/04* (2006.01)  
*A24B 15/14* (2006.01)

(52) **U.S. Cl.**

CPC ..... *A24B 3/14* (2013.01); *A24B 3/04* (2013.01); *A24B 15/12* (2013.01); *A24B 15/14* (2013.01)

(58) **Field of Classification Search**

CPC .. A24B 3/14; A24B 15/14; A24B 3/04; A24B 15/12

See application file for complete search history.

(56) **References Cited**

U.S. PATENT DOCUMENTS

|                 |         |             |
|-----------------|---------|-------------|
| 3,076,729 A     | 2/1963  | Garbo       |
| 4,306,578 A     | 12/1981 | Schmidt     |
| 4,319,593 A     | 3/1982  | Pinion      |
| 4,542,755 A     | 9/1985  | Selke       |
| 4,880,018 A     | 11/1989 | Graves, Jr. |
| 8,007,637 B2    | 8/2011  | Liu         |
| 8,136,533 B2    | 3/2012  | Mua         |
| 8,833,681 B2    | 9/2014  | Tarverdi    |
| 2008/0142027 A1 | 6/2008  | Ehling      |
| 2008/0216854 A1 | 9/2008  | Nicholls    |
| 2008/0245378 A1 | 10/2008 | Liu         |

FOREIGN PATENT DOCUMENTS

|    |             |         |
|----|-------------|---------|
| CN | 85105001    | 11/1989 |
| CN | 85104502    | 10/1990 |
| CN | 100443002   | 12/2008 |
| CN | 102640979   | 8/2012  |
| CN | 103005658   | 4/2013  |
| CN | 103798948   | 5/2014  |
| CN | 102669809   | 7/2014  |
| CN | 103734893   | 11/2015 |
| CN | 103783651   | 4/2016  |
| EA | 015099      | 6/2011  |
| EP | 1872670     | 1/2008  |
| GB | 1203940     | 9/1970  |
| JP | 53-133700   | 11/1978 |
| JP | 61-052269   | 3/1986  |
| JP | 2009-504166 | 2/2009  |
| JP | 2012-530857 | 12/2012 |
| KZ | 4908 B      | 9/1998  |
| RU | 2346629     | 2/2009  |
| UZ | 2219 C      | 10/2002 |

OTHER PUBLICATIONS

Office Action issued in Europe for Application No. 15730781.0 dated Feb. 5, 2018 (5 pages).

Office Action issued in China for Application No. 20150031815.9 dated Nov. 3, 2017 (19 pages). English translation included.

PCT Search Report and Written Opinion for PCT/EP2015/063979 dated Sep. 2, 2015 (11 pages).

Office Action in Kazakhstan for Application No. 2017/0032 dated May 18, 2018 (8 pages). English translation included.

Office Action in Philippines for Application No. 1-2016-502032 dated Jul. 4, 2018 (6 pages).

Office Action issued in China for Application No. 201580031815.9 dated Jul. 17, 2018 (26 pages). English translation included.

Office Action in Singapore for Application No. 11201610680Q dated Aug. 20, 2018 (7 pages).

(Continued)

*Primary Examiner* — Michael H. Wilson

*Assistant Examiner* — Dionne W. Mayes

(74) *Attorney, Agent, or Firm* — Muetting Raasch Group

(57) **ABSTRACT**

The invention relates to a reconstituted tobacco sheet having a basis weight of less than about 230 grams per square metre and comprising tobacco stem or tobacco stalk refined fibres having an average length of at least about 200 micrometres and tobacco cast leaf material. There is further provided a method of making a reconstituted tobacco sheet, the method comprising providing tobacco stems and conditioning the tobacco stems such that their moisture content is increased to at least about 40% Oven Volatiles (OV). The tobacco stems are processed in a twin screw extruder to so as to obtain a pulp suspension having a Schop-per-Riegler index of at least about 30 degrees and comprising tobacco stem or tobacco stalk refined fibres having an average length of at least about 200 micrometres. This pulp suspension is combined with tobacco cast leaf material to obtain a slurry and a sheet is formed from this slurry.

**11 Claims, No Drawings**

(56)

**References Cited**

**OTHER PUBLICATIONS**

Jian, Zeng, "Effect of Pulping on the Properties of the Paper Prepared from Tobacco Stem", Chemistry and Industry of Forest Products, vol. 32, No. 5, pp. 101-105, Oct. 2012. English translation included.

European Search Report for Application No. 14173740.3 dated Dec. 3, 2014 (6 pages).

Database WPI Jan. 1979 (Jan. 1979), Thomson Scientific, London, GB, AN 1979-010958 XP002733281, Nishida H.; OE H: "Low Bulk Density Sheet Tobacco Prod'n.—By Dispersing Tobacco Fibres, Accumulating on Running Conveyor, Moulding, Impregnating and Drying", & JP S 53 13370 A (Japan Tobacco & Salt Public) Nov. 21, 1978 (Nov. 21, 1978) "Abstract".

Office Action issued in China for Application No. 201580031815.9 dated May 15, 2019 (24 pages). English translation included.

Zhan Huaiyu, "Pulping Principle and Engineering", China Light Industry Pres, 3<sup>rd</sup> Edition, 4 pages. (English translation included), Jan. 31, 2009.

Wu Shubin, "Water Pollution Control and Treatment Technology in Paper Industry", Chemical Industry Press, 1<sup>st</sup> Edition, 3 pages. (English translation included). May 31, 2001.

Office Action issued in Japan for Application No. 2016-574920 dated Jul. 4, 2019 (18 pages). English translation included.

## RECONSTITUTED TOBACCO SHEETS AND RELATED METHODS

This application is a U.S. National Stage Application of International Application No. PCT/EP2015/063979, filed Jun. 22, 2015, which was published in English on Dec. 30, 2015, 2015, as International Publication No. WO 2015/197554 A1. International Application No. PCT/EP2015/063979 claims priority to European Application No. 14173740.3 filed Jun. 24, 2014.

The present invention relates to a reconstituted tobacco sheet and a method of making such reconstituted tobacco sheet. Further, the invention relates to tobacco products incorporating the reconstituted tobacco sheets.

There are several known methods for making reconstituted tobacco sheet. These several known methods may include processing tobacco material such as tobacco stems, tobacco stalks, leaf scraps and tobacco dust, which are produced during the manufacturing processes of tobacco products. Such manufacturing processes where the tobacco material may derive include stemming, aging, blending, cutting, drying, cooling, screening, sieving, shaping or packaging operations.

One of the known methods is to ground tobacco stems to a fine powder and then mix the tobacco stems with tobacco dust, guar gum, and water to form an aqueous slurry. This aqueous slurry may be then cast and dried to form a reconstituted tobacco sheet. However, this type of reconstituted tobacco sheet has a low tensile strength. In order to improve this characteristic of the reconstituted tobacco sheet, a non-tobacco cellulose, for example in the form of wood cellulose fibres, is usually added to the slurry as a binder. But, the presence of a non-tobacco ingredient is generally undesirable due to the increase in cost and negative impact on flavour attributed to this ingredient.

In other known methods, tobacco materials are mixed in an agitated tank with water to obtain a pulp. The soaking and mixing of the tobacco in the tank with water causes the water soluble components of the tobacco to dissolve into the liquid, creating a tobacco-flavoured liquid or tobacco juice. This tobacco-flavoured liquid subsequently needs to be separated from the non-soluble portion of the tobacco before further processing. By way of example, the pulp may be compressed or processed using a centrifuge to remove the tobacco-flavoured liquid containing the water-soluble components. The non-water-soluble portion then subsequently undergoes a paper-making process (for example, using a Fourdrinier machine) to form a base web. As is known, a Fourdrinier machine typically includes a forming section, a press section and a drying section. In the forming section, which comprises a plastic fabric mesh conveyor belt often referred to as a "wire", as it was once woven from bronze, the pulp is drained to create a continuous paper web. Subsequently, this wet web is fed onwards to the press section, where the excess water is squeezed out of the web. Finally, the pressed web is conveyed on through a heated drying section. The tobacco-flavoured liquid is also subjected to further processing using an evaporation operation to form a concentrated liquor, which may be added back to the base web in order to at least partly restore flavour to the base web that would otherwise be lost. Dried reconstituted tobacco sheet typically displays a relatively limited tensile strength. In addition, the methods described above also have the drawback of high energy consumption due to the evaporation process. Further, even a partial loss of tobacco soluble components can have an undesirable impact on flavour.

Therefore, it would be desirable to provide a method of making a reconstituted tobacco sheet with a greater tensile strength compared with the reconstituted tobacco sheets obtainable from existing methods and without the need for the sheet to be reinforced with undesirable non-tobacco cellulosic materials as binders, such that the resulting reconstituted tobacco sheet is better suited for withstanding mechanical stresses during the manufacture of tobacco products from the sheet. Further, it would be desirable to provide a method of making a reconstituted tobacco sheet that allows for a reduced energy consumption compared with known processes. At the same time, it would be desirable to provide a method of making a reconstituted tobacco sheet by which the tobacco flavour sources are better preserved and by virtue of which the resulting reconstituted tobacco sheet has an increased filling power. The term "filling power" is used throughout this specification to refer to the volume of space taken up by a given weight or mass of a tobacco material. The greater the filling power of a tobacco material, the lower the weight of the material required to fill a tobacco rod of standard dimensions. The values of filling power are expressed in terms of corrected cylinder volume (CCV), which is the cylinder volume (CV) of the tobacco material at a reference moisture level of 12.5% oven volatiles. The cylinder volume (CV) may be determined using a Borgwaldt densimeter DD60 or DD60A type fitted with a measuring head for cut tobacco and a tobacco cylinder container.

In a suitable method for determining the value of CCV, a sample of the cut filler is placed in the tobacco cylinder container of the Borgwaldt densimeter and subjected to a load of 2 kg for 30 seconds. The height of the sample after the loading time has expired is measured and this is converted to a cylinder volume using the formula:

$$CV = \frac{r^2 \cdot h \cdot \pi}{SW \cdot 10}$$

where  $r$  is the cylinder radius (3.00 cm for the densimeter indicated above),  $h$  is the height of the sample after the loading time has expired and  $SW$  is the weight of the sample. The measured  $CV$  is then converted to a corrected value of CCV at the reference moisture level value (ROV) of 12.5% oven volatiles, using the formula:

$$CCV = (OV - ROV) \cdot f \cdot CV$$

where  $OV$  is the actual % oven volatiles of the sample of tobacco stems and  $f$  is a correction factor (0.4 for the test indicated).

The term "% Oven Volatiles" (%  $OV$  or percent  $OV$ ) is used to refer to the moisture content of the tobacco stems. It is determined by measuring the percentage weight loss from the stems upon drying a sample of the stem material in an oven at  $100 \pm 1$  degrees Centigrade ( $^{\circ}$  C.) for 3 hours  $\pm 0.5$  minutes. In practice, it is assumed that a significant majority of the weight loss from the stems results from the evaporation of moisture. It should be noted that, on an absolute basis, the values of moisture content determined by oven drying may be greater than the results of water content analysis when using a specific method such as ISO 6488 (Karl Fischer method). The difference is sample-type dependent and is due to the loss of volatile materials other than water from the tobacco material during oven drying.

The term "L/D ratio" is used throughout this specification to identify the ratio between the length ( $L$ ) and the diameter

(D) of each screw in the pair of screws of a twin-screw extruder used for processing the stem material.

According to a first aspect of the invention there is therefore provided a method of making a reconstituted tobacco sheet, comprising providing tobacco stems or stalks or a mixture thereof and conditioning the tobacco stems or stalks (or their mixture) such that their moisture content is increased to at least about 40% Oven Volatiles (OV). The conditioned tobacco stems or stalks are processed in a twin screw extruder so as to obtain a pulp suspension having a Schopper-Riegler index of at least about 30 degrees and comprising tobacco stem or stalk fibres having a length of at least about 200 micrometres. The pulp suspension comprising the tobacco stem or tobacco stalk refined fibres is combined with tobacco cast leaf material to obtain a slurry.

A sheet is then formed from this slurry.

Further, according to a second aspect of the invention, there is provided a reconstituted tobacco sheet having a basis weight of less than about 230 grams per square metre and comprising tobacco stem or tobacco stalk refined fibres having an average length of at least about 200 micrometres.

It will be appreciated that any features described with reference to one aspect of the present invention are equally applicable to any other aspect of the invention.

The term "tobacco products" is used throughout this specification to refer to both combustible smoking articles and to smoking articles in which an aerosol forming substrate, such as tobacco, is heated rather than combusted. Combustible smoking articles, such as cigarettes, generally comprise shredded tobacco (usually in cut filler form) surrounded by a paper wrapper forming a tobacco rod. The shredded tobacco can be a single type of tobacco or a blend of two or more types of tobacco. A cigarette is employed by a consumer by lighting one end thereof and burning the shredded tobacco rod. The consumer then receives mainstream smoke by drawing on the opposite end (mouth end or filter end) of the cigarette. In heated smoking articles, the aerosol is generated by heating the aerosol forming substrate. Known heated smoking articles include, for example, smoking articles in which an aerosol is generated by electrical heating or by the transfer of heat from a combustible fuel element or heat source to an aerosol forming substrate. During smoking, volatile compounds are released from the aerosol forming substrate by heat transfer from the heat source and entrained in air drawn through the smoking article. As the released compounds cool, they condense to form an aerosol that is inhaled by the consumer. Also known are smoking articles in which a nicotine-containing aerosol is generated from a tobacco material, tobacco extract, or other nicotine source, without combustion, and in some cases without heating, for example through a chemical reaction. In the present specification, the term "stalk" is used to refer to the main structural portion of the tobacco plant that remains after the leaves, including the stem and lamina, have been removed. The stalk supports the tobacco leaves and connects them to the roots of the plant and has a high cellulosic content.

The term "stem" is used herein to refer to the structural portion of the tobacco plant connecting the lamina to the stalk, and also to the veins or ribs that extend through the leaves between the lamina portions. In the context of the present invention, the term "stem" does not encompass the term "stalk" and the stems and stalk of the tobacco plant are considered as distinct portions.

The term "refine" is used throughout the specification to mean that the tobacco stems or tobacco stalks in the liquid dispersion are subjected to a mechanical treatment that

modifies the fibres of the stem material so that they can be formed into a sheet. For example, conical refiners or disc refiners of the type commonly used for wood pulp refining in the paper industry may be used to this purpose. This 5 mechanical process is understood to exert an abrasive and bruising action on the tobacco stem fibres such that they are broken, deformed, delaminated and declustered, yet not so damaged that they lose too much of their strength. Accordingly, hair-like, thin and elongated tobacco stem or tobacco 10 stalk "refined fibres" may be obtained from tobacco stems. These tobacco stem or tobacco stalk "refined fibres" are pliable and have greater surface area. This is understood to 15 significantly improve inter-fibre bonding ability, in that it appears to favour the formation of hydrogen bonds between overlying strands.

By the term "fibre length", reference is made throughout the specification to the major dimension of a fibre obtained by refining tobacco stems or stalks by a method according to the invention. More particularly, reference is generally made 20 to the average value of the fibre length as measured on a sample of the tobacco stem or stalk fibres. Average fibre length may be assessed experimentally by several methods. For example, fibre length may be measured by microscope analysis.

The term "cast leaf" is used herein to refer to a process that is well known in the art and that is based on casting a slurry comprising ground tobacco particles and a binder (for example, guar) onto a supportive surface, such as a belt conveyor, drying the slurry and removing the dried sheet 25 from the supportive surface. The term "tobacco cast leaf material" is used herein to refer to the portions of the tobacco leaf and to the recoverable fine material generated during processing (for example, tobacco dust) that are 30 normally used in a conventional cast leaf process.

The term "freeness" is used throughout this specification to refer to the drainability of a pulp product. The "freeness" is defined by the 2014 publication of the International Standard ISO 5267-1 entitled: Determination of Drainability Part—1: Schopper-Riegler Method. The Schopper-Riegler 35 test is designed to provide a measure of the rate at which a dilute suspension of pulp may be dewatered. It has been shown that drainability is related to the surface conditions and swelling of the fibres, and constitutes a useful index of the amount of mechanical treatment to which the pulp has 40 been subjected. Therefore, it shall be clear for the skilled reader that, by indicating the value of freeness or drainability 45 of a pulp obtained by a refining operation, reference is indirectly being made to the intensity and amount of mechanical treatment (for example, in terms of net energy input) to which said pulp has been subjected in the refining 50 operation. Freeness (drainability) may be expressed in degrees Schopper-Riegler. The pulp is prepared in accordance with the test conditions defined in the above identified ISO standard. A volume of 1000 ml of the prepared pulp is 55 poured into the drainage chamber. The discharge from the bottom and side orifices is collected. The filtrate from the side orifice is measured in a special cylinder, graduated in SR degrees. A discharge of 1000 millilitres corresponds to 0 degrees Schopper-Riegler while a discharge of 0 millilitres 60 corresponds to 100 degrees Schopper-Riegler.

The term "tensile strength" is used throughout the specification to indicate a measure of the force required to stretch a reconstituted tobacco sheet until it breaks. More specifically, the tensile strength is the maximum tensile force per unit width that the sheet material will withstand before 65 breaking and is measured in the machine direction of the sheet material. It is expressed in units of Newtons per meter

of material (N/m). Tests for measuring the tensile strength of a sheet material are well known. A suitable test is described in the 2014 publication of the International Standard ISO 1924/2 entitled "Paper and Board—Determination of Tensile Properties Part—2: Constant Rate of Elongation Method".

The test utilises tensile testing apparatus which is designed to extend a test piece of given dimensions at an appropriate constant rate of elongation and to measure the tensile force and, if required, the elongation produced. Each test piece of sheet material is held in two clamps, the separation of which is adjusted at a specified rate. For example, for a 180 millimeters test length the rate is 20 millimeters per minute. The tensile force is measured as a function of elongation and the test is continued until the test piece ruptures. The maximum tensile force is measured, as well as the elongation at break.

The tensile strength of the material may be calculated from the following equation in which  $S$  is the tensile strength in N/m,  $\bar{F}$  is the mean tensile force in Newton and  $w$  is the width of the test piece in metres:

$$S = \frac{\bar{F}}{w}$$

A reconstituted tobacco sheet according to the invention has a basis weight of less than about 230 grams per square metre. In addition, a reconstituted tobacco sheet according to the invention has preferably a basis weight of at least about 80 grams per square metre. More preferably, the basis weight is at least about 100 grams per square metre. In some preferred embodiments, the basis weight is about 155 grams per square metre.

Because the basis weight of the reconstituted tobacco sheet is reduced, compared to reconstituted tobacco sheets obtained by certain known methods, the filling power of the reconstituted tobacco sheet may advantageously be improved. Thus, the overall tobacco weight in smoking articles may advantageously be reduced.

Further, a reconstituted tobacco sheet according to the invention is formed from tobacco stem or stalk refined fibres having an average length of at least about 200 micrometres. A tobacco stem or tobacco stalk refined fibre average length of at least about 200 micrometres has been found to ensure satisfactory inter-fibre bonding and, as a consequence, to favour the formation of a sheet material having desirable mechanical properties. Preferably, the stem or stalk refined fibres have an average length of at least about 300 micrometres.

In addition, the stem or stalk refined fibres preferably have an average length of less than about 1200 micrometres. It has been found that tobacco stem or tobacco stalk refined fibres having such fibre length may effectively contribute to improving the tensile strength of a reconstituted tobacco sheet formed from them. Without being bound to theory, it is thought that tobacco stem or tobacco stalk refined fibres having such fibre length provide a suitable amount of surface area for inter-fibre bonding.

Even more preferably, the tobacco stem or tobacco stalk refined fibres have an average length of less than about 1000 micrometres. In some particularly preferred embodiments, the stem or stalk refined fibres have an average length of about 400 micrometres.

The reconstituted tobacco sheet contains at least about 10 percent by weight of the dry sheet of tobacco stem or

tobacco stalk refined fibres. Preferably, the tobacco stem or tobacco stalk refined fibres account for at least about 20 percent by weight of the dry sheet. More preferably, the tobacco stem or tobacco stalk refined fibres account for at least about 30 percent by weight of the dry sheet. Even more preferably, the tobacco stem or tobacco stalk refined fibres account for at least about 40 percent by weight of the dry sheet. In addition, or as an alternative, the reconstituted tobacco sheet contains less than about 80 percent by weight of the dry sheet of tobacco stem or tobacco stalk refined fibres. In some preferred embodiments, the tobacco stem or tobacco stalk refined fibres account for from about 20 percent by weight of the dry sheet to about 50 percent by weight of the dry sheet, even more preferably from about 40 percent by weight of the dry sheet to about 50 percent by weight of the dry sheet. It has surprisingly been found that higher contents of tobacco stem or tobacco stalk refined fibres having an average length of at least about 200 micrometres may result in a significantly increased tensile strength of the reconstituted tobacco sheet, as will be shown by the Examples below.

The reconstituted tobacco sheet may have a tensile strength of at least about 196 Newtons per meter. Preferably, the reconstituted tobacco sheet has a tensile strength of at least about 245 Newtons per meter. More preferably, the reconstituted tobacco sheet has a tensile strength of at least about 294 Newtons per meter. Such improved values of tensile strength make the reconstituted tobacco sheet according to the present invention particularly suitable for subsequent operations involving mechanical stresses.

The reconstituted tobacco sheets according to the invention find particular application in the manufacture of tobacco products, including combustible smoking articles and smoking articles in which an aerosol forming substrate, such as tobacco, is heated rather than combusted. In more detail, after forming, a reconstituted tobacco sheet can be dried and further shaped and cut. In a preferred embodiment, the reconstituted tobacco sheet is cut to form strips that are cut with other forms of tobacco strips to form a mixed cut filler that can be used to manufacture a reconstituted tobacco product, such as a tobacco rod or an aerosol forming substrate to be heated rather than combusted. Alternatively, the reconstituted tobacco sheet may be cut independently to form a reconstituted tobacco cut filler component, and then the reconstituted tobacco cut filler component can then be blended with other filler components. In particular, a reconstituted tobacco material formed from a reconstituted tobacco sheet according to the present invention can be blended with other tobaccos to form a cut filler. Such cut filler may include, but is not limited to, shreds of flue-cured tobacco, Burley tobacco, Maryland tobacco, Oriental tobacco, rare tobacco, specialty tobacco, reconstituted tobacco, expanded tobacco and the like. The cut filler can also include conventional additives, for example humectants, such as glycerine and propylene glycol.

In a method of making a reconstituted tobacco sheet according to the invention, tobacco stems or stalks are conditioned such that their moisture content is increased to at least about 40 percent OV. Preferably, the tobacco stems are conditioned such that their moisture content is increased to at least about 50 percent OV. In addition, or as an alternative, the tobacco stems are conditioned such that their moisture content is increased to less than about 90 percent OV. Preferably, the tobacco stems or stalks are conditioned such that their moisture content is increased to less than about 80 percent OV. In some preferred embodiments, the tobacco stems or stalks are conditioned such that their

moisture content is increased to from about 75 percent OV to about 80 percent OV. In other preferred embodiments, the tobacco stems are conditioned such that their moisture content is increased to from about 40 percent OV to about 60 percent OV. For example, the tobacco stems are conditioned such that their moisture content is increased to about 50 percent OV.

The conditioned stems are processed in a twin screw extruder so as to obtain a pulp suspension having a Schopper-Riegler index of at least about 30 degrees and comprising tobacco stem or tobacco stalk refined fibres having an average length of at least about 200 micrometres. This pulp suspension is combined with tobacco cast leaf material to obtain a slurry, from which a sheet is formed.

Because substantially all the soluble fraction (also often referred to as "tobacco juice") is kept within the stem material, most flavour sources are advantageously preserved. At the same time, because there is no need to concentrate by evaporation a liquid phase separated from the non-soluble portion of the tobacco stems, as is the case with certain known processes, the overall energy consumption associated with the method according to the present invention is advantageously reduced. Further, the need to introduce non-tobacco cellulosic material is substantially eliminated altogether, because the tobacco stem fibres obtained by processing by extrusion the tobacco stem material provide sufficiently solid inter-fibre bonds. In general, this results in an improved tensile strength of reconstituted tobacco sheets obtainable by the method. Further, the higher content of fibrous material may result in a particularly rough, wavy surface texture of the reconstituted tobacco sheet. Thus, the filling power of the reconstituted tobacco may be advantageously increased.

Preferably, the tobacco stems are processed in the extruder to obtain a pulp suspension comprising tobacco stem or tobacco stalk refined fibres having an average length of less than about 1200 micrometres. More preferably, the tobacco stems are processed in the extruder to obtain a pulp suspension comprising tobacco stem or tobacco stalk refined fibres having an average length of less than about 1000 micrometres. In a preferred embodiment, the tobacco stems are processed in the extruder to obtain a pulp suspension comprising tobacco stem or tobacco stalk refined fibres having an average length from about 200 micrometres to about 800 micrometres.

Preferably, the tobacco stems are processed in the extruder to obtain a pulp suspension having a Schopper-Riegler index of at least about 50 degrees.

Preferably, the step of processing the conditioned stems in the extruder is carried out at a temperature of at least about 50 degrees C. More preferably, the step of processing the conditioned stems or stalks in the extruder is carried out at a temperature of at least about 60 degrees C. In addition, or as an alternative, the step of processing the conditioned stems or stalks is carried out at a temperature of less than about 140 degrees C. Preferably, the step of processing the conditioned stems or stalks in the extruder is carried out at a temperature of less than about 100 degrees C. In some preferred embodiments, the step of processing the conditioned stems in the extruder is carried out at a temperature of from about 60 degrees C. to about 100 degrees C.

In preferred embodiments, different heated sections of the extruder are maintained at different temperatures, such that the stem material being processed is exposed to an increasing temperature as it travels along the extruder. By way of example, in a first heated section of the extruder, the tobacco stems or stalks are processed at a temperature lower than the

temperature in a second heated section of the extruder. In some embodiments, the cooler heated section of the extruder is upstream of the second heated section of the extruder. In other embodiments, the cooler heated section of the extruder is downstream of the second heated section of the extruder.

Preferably, in a first section of the extruder, the tobacco stems are processed at a temperature of at least about 50 degrees C. In addition, or as an alternative, in a first section of the extruder, the tobacco stems or tobacco stalks are processed at a temperature of less than about 95 degrees C. In a second section of the extruder, the tobacco stems or tobacco stalks are processed at a temperature of at least about 90 degrees C. In addition, or as an alternative, in a second section of the extruder, the tobacco stems or tobacco stalks are processed at a temperature of less than about 110 degrees.

In some embodiments, the first and second heated sections of the extruder may be separated by a non-heated section of the extruder. Further, the extruder may comprise one or more additional non-heated section upstream or downstream of the first and second heated sections. In addition, or as an alternative, the extruder may comprise one or more additional heated sections.

In preferred embodiments, the step of processing the tobacco stems or tobacco stalks comprises a first and a second steps of passing the tobacco stem or stalk material through the twin screw extruder. Without wishing to be bound to theory, it has been observed that the first extruding step substantially turns the conditioned tobacco stems or tobacco stalks into a rather coarse pulp, wherein stem or stalk fibres have not yet been properly separated, whereas the second extruding step substantially turns the coarse pulp obtained from the first extruding step into a much finer pulp suspension.

Preferably, the tobacco stems or tobacco stalks are extruded to obtain a pulp suspension having a Schopper-Riegler index of at least about 50 degrees after the second passing step.

In some preferred embodiments, the tobacco stems or tobacco stalks are extruded to obtain a pulp suspension having a Schopper-Riegler index of at least about 30 degrees after the first passing step and of at least about 60 degrees after the second passing step.

Preferably, the step of processing the conditioned stems or stalks is carried out in a twin screw extruder comprising at least a first and a second conveying sections adapted to advance the material being processed along an axial direction of the extruder and at least a kneading section adapted to restrict the flow of the material being processed along the axial direction and to exert a kneading and shearing action on the stems, wherein the at least one kneading/shearing section is located between the first and the second conveying sections.

Preferably, the twin extruder has a L/D ratio of from 25 to 70. In addition, or as an alternative, the at least one kneading section extends over a length of at least 10 D.

The invention will be further described with reference to the following, non-limiting examples.

#### COMPARATIVE EXAMPLE

A reconstituted tobacco sheet was prepared according to a conventional cast leaf process with the following composition:

##### Tobacco Material:

Lamina dust: 66 percent by dry weight  
Ground stem: 34 percent by dry weight

## Binder:

Guar: 8 parts by dry weight per 100 parts of dry tobacco material

The dry tobacco material was fed to a grinder where it was dry ground and screened and subsequently contacted with an aqueous medium including guar as the binder in a high-shear mixer to form a tobacco slurry. The tobacco slurry was then cast onto a moving endless belt. The cast slurry was subsequently passed through a drying assembly to remove moisture so as to form a reconstituted tobacco sheet. Finally, the sheet was removed from the belt with a doctor blade.

A reconstituted tobacco sheet was obtained with a basis weight of  $12.5 \pm 0.5$  grams per square foot (about 135 grams per square metre) and a tensile strength of about 25 kgf/m (about 245 N/m).

## Example 1

Tobacco stem refined fibres were prepared by an embodiment of a method in accordance with the present invention. In more detail, tobacco stems were conditioned to moisture content of about 50 percent OV. Subsequently, the conditioned tobacco were processed with two subsequent passes in a twin-screw extruder with an L/D ratio of 48 and a screw diameter of 53 mm. The screw profile was composed of a sequence of conveying sections and kneading (restrictive) sections. In more detail, the screw profile included 6 kneading sections, for an overall length of kneading section of about 20 D. Consecutive kneading sections were separated by conveying zones. The first two kneading sections were provided as reverse screw elements with large grooves. The following kneading sections were provided as kneading elements with positive, neutral or negative pitches, as well as reverse screw elements. The kneading elements were bilobal, but monolobal or trilobal could also have been used.

## First Pass

The conditioned tobacco stems were fed to the extruder at a feed rate of 25 kg/hour. The extruder screw speed was set at 250 rpm. The temperature along the screw extruder was regulated in order to prevent the stems to reach a temperature above 100 degrees C. In more detail, in a first section of the extruder, the temperature was set at about 90 degrees C. In a second section of the extruder downstream of the first section, the temperature was set at about 100 degrees C. The moisture of the stems at the exit of the extruder after the first pass was about 45 percent OV. The freeness (drainability) measured on the stems at the exit of the extruder after the first pass was about 62 degrees Schopper-Riegler.

## Second Pass

The conditioned tobacco stems were fed to the extruder at a feed rate of 25 kg/hour. The extruder screw speed was set at 250 rpm. The temperature along the screw extruder was regulated in order to prevent the stems to reach a temperature above 100 degrees C. In more detail, in a first section of the extruder, the temperature was set at about 90 degrees C. In a second section of the extruder downstream of the first section, the temperature was set at about 100 degrees C. The moisture of the stems at the exit of the extruder after the first pass was about 37 percent OV. The freeness (drainability) measured on the stems at the exit of the extruder after the first pass was about 75 degrees Schopper-Riegler.

Tobacco stem refined fibres having a average length of about 350 micrometres were obtained. The tobacco stem refined fibres thus obtained were mixed with humectants and tobacco dust and binder to form a slurry, which was then cast to form a sheet and let dry.

## Example 2

Tobacco stem refined fibres were prepared by an alternative embodiment of a method in accordance with the present invention. In more detail, tobacco stems were conditioned to moisture content of about 50 percent OV. Subsequently, the conditioned tobacco were processed with two subsequent passes in a twin-screw extruder with an L/D (length to diameter) ratio of 28 and a screw diameter of 42 mm. The screw profile was composed of a sequence of conveying sections and kneading (restrictive) sections. In more detail, the screw profile included 6 kneading sections, for an overall length of kneading section of about 19 times the screw diameter D. Consecutive kneading sections were separated by conveying zones. The kneading sections were provided as kneading elements of different sizes with positive or negative pitches, as well as reverse screw elements. The kneading elements were bilobal, but monolobal or trilobal could also have been used. The reverse screw elements were without grooves.

## First Pass

The conditioned tobacco stems were fed to the extruder at a feed rate of 25 kg/hour. The extruder screw speed was set at 250 rpm. In the downstream section of the screw extruder the temperature was regulated in order to prevent the stems to reach a temperature above 100 degrees C. The moisture of the stems at the exit of the extruder after the first pass was about 44 percent OV. The freeness (drainability) measured on the stems at the exit of the extruder after the first pass was about 33 degrees Schopper-Riegler.

## Second Pass

The conditioned tobacco stems were fed to the extruder at a feed rate of 25 kg/hour. The extruder screw speed was set at 250 rpm. In the downstream section of the screw extruder the temperature was regulated in order to prevent the stems to reach a temperature above 100 degrees C. The moisture of the stems at the exit of the extruder after the first pass was about 40 percent OV. The freeness (drainability) measured on the stems at the exit of the extruder after the first pass was about 52 degrees Schopper-Riegler.

Tobacco stem refined fibres having an average length of about 400 micrometres were obtained. The tobacco stem refined fibres thus obtained were mixed with humectants and tobacco dust and binder to form a slurry, which was then cast to form a sheet and let dry.

## Example 3

A reconstituted tobacco sheet was prepared by a method according to the present invention as described above with reference to Example 2 with the following composition:

## Tobacco Material:

Lamina dust: 62 percent by dry weight

Refined stem fibres: 30 percent by dry weight

## Binder:

Guar: 8 parts by dry weight per 100 parts of dry tobacco material

A reconstituted tobacco sheet was obtained with a basis weight of about 160 grams per square metre) and a tensile strength (about 300 N/m).

## Example 2

A reconstituted tobacco sheet has been prepared by a method according to the present invention with the following composition:

## 11

## Tobacco Material:

Lamina dust: 57 percent by dry weight

Refined stem fibres: 43 percent by dry weight.

## Binder:

Guar: 8 parts by dry weight per 100 parts of dry tobacco material.

A reconstituted tobacco sheet was obtained with a basis weight of about 150 grams per square metre and a tensile strength of about 340 N/m.

The invention claimed is:

1. A method of making a reconstituted tobacco sheet, comprising:

providing tobacco stems or tobacco stalks or a mixture thereof;

conditioning the tobacco stems or tobacco stalks such that their moisture content is increased to from about 40%

Oven Volatiles (OV) to about 60% Oven Volatiles (OV);

processing the conditioned tobacco stems or tobacco stalks in a twin screw extruder to so as to obtain a pulp suspension having a Schopper-Riegler index of at least about 30 degrees and comprising tobacco stem or tobacco stalk refined fibres having an average length of at least about 200 micrometres;

combining the pulp suspension with tobacco cast leaf material to obtain a slurry; and

forming a sheet from the slurry.

2. A method according to claim 1, wherein the conditioned tobacco stems or tobacco stalks are extruded to obtain a pulp suspension containing tobacco stem or tobacco stalk refined fibres having an average length of less than about 1200 micrometres.

3. A method according to claim 2, wherein the step of processing the conditioned stems or stalks is carried out at a temperature of at least about 50 degrees C.

4. A method according to claim 1, wherein the step of processing the conditioned stems or stalks is carried out at a temperature of at least about 50 degrees C.

## 12

5. A method according to claim 4, wherein the step of processing the conditioned stems or stalks is carried out in a twin screw extruder comprising at least a first and a second conveying sections adapted to advance the material being processed along an axial direction of the extruder and at least a kneading section adapted to restrict the flow of the material being processed along the axial direction and to exert a kneading and shearing action on the stems, wherein the at least one kneading section is located between the first and the second conveying sections.

6. A method according to claim 1, wherein the step of processing the conditioned tobacco stems or tobacco stalks comprises one or more passes of the conditioned tobacco stems or tobacco stalks through the twin screw extruder.

7. A method according to claim 1, wherein the step of processing the conditioned stems or stalks is carried out in a twin screw extruder comprising at least a first and a second conveying sections adapted to advance the material being processed along an axial direction of the extruder and at least a kneading section adapted to restrict the flow of the material being processed along the axial direction and to exert a kneading and shearing action on the stems, wherein the at least one kneading section is located between the first and the second conveying sections.

8. A method according to claim 7, wherein the twin screw extruder has a Length/Diameter ratio of from 25 to 70.

9. A method according to claim 8, wherein the at least one kneading section extends over a length of at least 10 times the screw diameter.

10. A method according to claim 7, wherein the at least one kneading section extends over a length of at least 10 times the screw diameter.

11. A reconstituted tobacco sheet obtainable by a method according to claim 1.

\* \* \* \* \*